

# UNITED STATES PATENT OFFICE.

GEORGE L. PRICHARD, OF PORT ARTHUR, TEXAS, ASSIGNOR TO GULF REFINING COMPANY, OF PITTSBURGH, PENNSYLVANIA, A CORPORATION OF TEXAS.

## UTILIZATION OF ACID-COKE.

1,290,345.

Specification of Letters Patent.

Patented Jan. 7, 1919.

No Drawing.

Application filed May 2, 1917. Serial No. 166,007.

To all whom it may concern:

Be it known that I, GEORGE L. PRICHARD, a citizen of the United States, residing at Port Arthur, in the county of Jefferson and State of Texas, have invented certain new and useful Improvements in the Utilization of Acid-Coke, of which the following is a specification.

This invention relates to the utilization of acid coke; and it comprises a method of utilizing the coky matter from the treatment of mineral oils with sulfuric acid, wherein such coky matter is mingled with a heavy oil and kept in suspension by suitable agitating means, such as an air blast, and while so suspended is conveyed to a place of use by pumps or the like and at such place of use is burned while still in admixture with said heavy oil; all as more fully hereinafter set forth and as claimed.

As is well known, the customary method of "treating" mineral oils is to agitate the same with sulfuric acid. This has the effect of removing unsaturated hydrocarbons, benzenoid bodies, etc. After the treatment is complete, the sulfuric acid settles as "acid sludge." This sludge contains a considerable amount of oil which is separated and recovered by various methods. The oil so recovered is known as "acid oil" or sludge oil. The final oil-free product of these recovery methods is a hard, solid, coky mass, somewhat similar in physical properties to a very hard asphalt, or an asphalt concrete, and consisting in substance of grains or granules of coky carbon cemented together with asphalt or asphalt-like matter. It is ordinarily burnt for the sake of its fuel value. It still contains some acid and this renders its handling and utilization difficult; the difficulty being of course accentuated by the physical form of such material. It is the common practice to transfer this material, which may be hereinafter called acid coke, in cars or buckets, from the point of origin to the point of consumption, which is generally a furnace, such as a boiler furnace. It is sometimes fed into the furnaces by workmen handling it with shovels; but this is laborious and unsatisfactory. As stated, the material is very much like an asphalt physically. Sometimes the coky mass is delivered into bins from which it is allowed to flow into the furnace through large troughs while still hot enough to be

flowable. In the furnace it does not burn readily; imperfect combustion usually occurring with formation of large volumes of smoke. As acid coke is usually burnt, it is not only apt to create a nuisance but its combustible value is not well utilized and the operation is expensive because of the labor involved. And the whole equipment for delivering the material to the furnace must be either made of costly acid proof material or renewed frequently.

I have found that a satisfactory method of handling and utilizing this material is to commingle it with fuel oil which dissolves or softens the asphalt constituents and forms a mass or magma which can be pumped and handled. The mixture of fuel oil and acid coke can be burnt very satisfactorily with ordinary firing means, while the mixture is not corrosive, the oil enveloping the acid-carrying coke particles. Other cheap oils from the refinery may also be utilized. An advantageous mixture may be afforded by taking 1 part acid oil of 0.954 specific gravity, 1 part Texas asphaltum oil of about 0.9825 specific gravity and 1 part of acid coke of about 1.197 specific gravity.

The coke may be mingled with the oil in about the proportions specified, or in any other proportions which will give a flowable mixture, the oil being in a heated state, and the mixture kept in constant agitation by means of an air blast supplied to the mixing apparatus through a perforated pipe. Any other agitating means may be used, but air agitating is convenient and effective. The proportions and character of oil given above are merely indicative and refer to one particular acid coke. Other acid cokes of a somewhat drier character require somewhat more oil, while, on the other hand, a softer acid coke requires somewhat less. The hot agitated mixture may be conveyed to a point of use through any suitable conduit, such as iron or steel pipes, by means of ordinary pumps. As the requirements of fuel burning furnaces vary from time to time while it is inadvisable to stop or check the flow of the oil-coke mixture when once established, since this might permit settling and separation, it is in general advisable to have the agitating and conveying means equal to supplying the maximum demands of the furnaces and to establish a back flow of such excess or overflow.

as there may be to the point of beginning; or, in other words, the agitated mixture of oil and coke may be kept in cyclic circulation with withdrawal from the flow of the 5 amount required for firing. While the acid coke is a corrosive material *per se*, yet, when mingled with oil in the manner described, the mixture may be safely handled in iron or steel. The mixture should be kept in motion 10 from the point of manufacture to the point of discharge, but otherwise its treatment in no wise differs from that of any ordinary fluid residuum used for fuel purposes. At the burners it may be sprayed 15 or otherwise handled by any of the means commonly adopted for similar purposes in handling fuel oil. The mixture burns readily and perfect combustion may be secured without the usual large volume of smoke attending the combustion of the coke alone. Handling of the material by workmen is not necessary at any point.

What I claim is:—

1. The method of utilizing acid coke from 25 sludge acid which comprises mingling the

same with heated oil and burning the mixture.

2. The method of utilizing acid coke from sludge acid which comprises mingling the same with heated oil to form a flowable mixture, transporting it to a point of use under constant agitation and burning the mixture.

3. The method of utilizing acid coke from sludge acid which comprises mingling such 35 acid coke with sufficient oil to make a flowable mixture, establishing and maintaining a cyclic flow of agitated mixture from the point of admixture to another point and back again and at an intermediate point 40 tapping off and burning a portion of the flowing mixture.

4. The method of utilizing acid coke from sludge acid which comprises softening the coky material with enough oil to render the 45 mixture fluid and delivering the softened material to a fire.

In testimony whereof, I affix my signature hereto.

GEORGE L. PRICHARD.